# EUROPEAN PATENT SPECIFICATION

(11) **EP 3 385 490 B1**
(45) Date of publication and mention of the grant of the patent: **17.01.2024**
(21) Application number: 18163303.3
(22) Date of filing: 22.03.2018
(51) Int. Cl.: E06B 9/15

(54) **SCREENING BODY WITH IMPROVED WEATHER RESISTANCE, UV RESISTANCE AND LAMINATION PROPERTIES**
ABSCHIRMKÖRPER MIT VERBESSERTER WITTERUNGSBESTÄNDIGKEIT, VERBESSERTEM UV-WIDERSTAND SOWIE VERBESSERTEN LAMINIERUNGSEIGENSCHAFTEN
CORPS D'ÉCRAN À RÉSISTANCE AMÉLIORÉE AUX INTEMPÉRIES, RÉSISTANCE AMÉLIORÉE AUX UV ET PROPRIÉTÉS DE STRATIFICATION AMÉLIORÉÉS

(30) Priority: 03.04.2017 DK PA201770241
(43) Date of publication of application: 10.10.2018
(73) Proprietor: VKR Holding A/S, 2970 Hørsholm (DK)
(72) Inventor: SØRENSEN, Martin, 8660 Skanderborg (DK); REMLER, Karina, 6715 Esbjerg N (DK); HØJ LAURSEN, Cecilie, 8370 Hadsten (DK)
(74) Representative: AWA Denmark A/S

(56) References cited:
- EP-A1- 1 048 817
- EP-A2- 0 806 541
- WO-A1-98/20225

## Description

The present invention relates to an improved screening body and a method for preparing the same. The screening body for a screening arrangement has improved properties in terms of ea. weather resistance, UV resistance and lamination properties.

### Background

Screening bodies are traditionally used for screening an aperture of a building structure, most often the light-admitting aperture of windows, but also of doors and other building openings. They are either installed to extend substantially vertically in a building façade, in an obliquely positioned roof window installed in an inclined roof surface, or as a horizontally extending cover for openings in a horizontal surface. When not screening the aperture, the screening body is normally rolled up on a roller bar accommodated in a top element of a screening arrangement.

The screening bodies can be used to block access to the aperture, to prevent light accessing the aperture and or/to help to moderate the temperature within a building.

In some forms, conventional screening bodies have a layered structure in which metal strips are bonded to a fabric web. One such system and a method of producing a metal foil - textile combination, particularly for use in roller shutters, is disclosed in EP1048817. The shutter slats are affixed to the web of the fabric using an adhesive. The document discloses that to manufacture a roller shutter, adhesive is applied at the contact surface of the metal profile or the woven fabric. The article is then shaped into a semi-finished product. The semi-finished units are later assembled, with the metal profiles and the woven fabric pressed against each other at their contact surfaces. The adhesive is activated and set by heating and cooling under pressure.

The lifetime of such devices is affected by the conditions to which they are exposed. For example, screening devices may be exposed to high and low temperature extremes. High temperature exposure and moisture exposure can cause accelerated degradation of the screening device as it promotes processes such as hydrolysis and oxidation within the components. Low temperature exposure can cause moisture trapped within the screening device to freeze. The expansion encountered as the water freezes can add stresses to the construction and can result in failure of parts of the screening device, particularly around adhesive interfaces.

The presence of moisture can also lead to further problems with screening devices. For example, water can cause hydrolysis of polymeric components as a result of the interaction of water molecules with the polymers thereby resulting in a breakdown of the molecular chains. UV radiation can also affect the screening devices, particularly as a result of polymer breakdown. UV radiation can stimulate the oxidation process which in turn can create free radicals which can cause breakdown of the polymer chains. In addition, air pollution and salt in the air, particularly in coastal environments, can increase rates of corrosion of the metallic components of screening devices.

These issues can affect the appearance of screening arrangements and, more seriously, can result in premature failure. It remains a challenge to provide a screening body that is better able to withstand at least some of these conditions.

### Summary of Invention

With this background it is an object to provide a screening body for a screening arrangement in which the screening body has improved lifetime due to improved resistance against one or more of the aforementioned causes of degradation. It is also an object to provide a screening arrangement comprising said screening body and a method of producing said screening body.

According to a first aspect of the present invention, there is provided a screening body for a screening arrangement including a top element defining a longitudinal direction, said screening body comprising a plurality of slats and a fabric layer having a top surface and a bottom surface, each slat extending in a longitudinal direction between two end edges and having first and second side edges parallel to the longitudinal direction, the screening body being adapted to be wound up in and rolled out from said top element in a direction perpendicular to said longitudinal direction to a screening position in which the screening body defines a general screening plane; in which each of the slats is composed of at least one metal strip connected to the fabric layer,
the screening body being characterised in that the at least one metal strip is coated on at least the side facing the fabric layer and that an adhesive layer binds the metal strip to the fabric layer.

It has surprisingly been found that the combination of the coating on the at least one metal strip and an adhesive composition used to bind the metal strip to the fabric layer results in a screening body that has improved properties. Without wishing to be bound by any theory, it is believed that by coating the at least one metal on the side facing the fabric layer, the metal is both protected from the adhesive and also primed to form a stronger bond with fabric through the adhesive.

In some arrangements, the at least first metal strip is arranged to contact the top surface of the fabric layer and a second metal strip is arranged to contact the bottom surface of the fabric layer. In this way, the screening body may have greater rigidity and strength.

According to the invention, the at least one first metal strip comprises aluminium. The at least one metal strip may comprise an alloy having an Al content in an amount of at least 90 wt% or more preferably at least 93 wt%, most preferred at least 95 wt%.

The coating of the at least one metal strip on at least the side facing the fabric layer comprises epoxy.

It has been observed that using coatings comprising epoxy groups gives rise to screening bodies with good adhesion properties to the aluminium and strong resistance to delamination, preferably the epoxy coating has aromatic groups. It is contemplated that the metal strip comprises additional layers such as primers etc. In the context of the present invention the coating is a layer of the metal strip that faces the fabric layer. The metal strips may have further coatings such as paint.

The adhesive composition comprises thermoplastic polyurethane or polyethylene terephthalate. More preferably, the adhesive composition comprises an aliphatic thermoplastic polyurethane, even more preferred an aliphatic polyether polyurethane. The adhesives are resistant to degradation, offer strong adhesion and are capable of percolating through the fabric.

Optionally, the adhesive layer may be applied to only one side of the fabric. In one embodiment the adhesive is applied to the bottom surface of the fabric layer facing the inside of a building when in use. Thereby the end product will have an improved appearance.

The adhesive composition may additionally comprise and/or possess a UV stabiliser.

In other embodiments the adhesive layer may be applied to the top surface of the fabric layer facing the exterior side of a building when in use. This embodiment is particularly preferred when the fabric layer is not UV stable, the adhesive layer comprising or being an UV stabilizer offers protection from UV light.

It was found that although the adhesive layer is only applied to one side of the fabric layer, the adhesion of one and/or two of the at least one coated metal strips is sufficient since the adhesive percolates through the fabric.

The fabric layer may comprise any material known in the art, preferably the fabric layer is made of acrylic, polyester, polyamide, glass fiber or a glass fiber reinforced fabric, most preferred the fabric layer is acrylic. The fabric layer is in a further preferred embodiment woven.

It is also contemplated that the fabric can be impregnated with and oil and/or water repellant such as fluorocarbon systems known in the art.

In further embodiments the porosity of the woven fabric is in the range of 50 to 500 mm, preferably 100 to 200, even more preferred 130 - 135, such as 133 when measured according to the Schmerber test in accordance to ISO 811. It is currently believed that the porosity or density of the fabric is important for improved adhesion. In some embodiments the fabric has a porosity that allows light through whilst the adhesive layer provides the darkening effect.

In some embodiments, the fabric layer comprises acrylic or polyester, the at least one first metal strip comprises aluminium in an amount of at least 90 wt%, the adhesive composition comprises a thermoplastic polyurethane and the coating comprises epoxy.

In embodiments where the fabric does not comprise glass fiber it is contemplated that the fabric layer is heated prior to being provided in step i. or that an adhesive composition is applied to the fabric under heating and is preferably allowed to cool down before being provided in step i. i.e. before another adhesive layer is applied to adhere the metal strip to the fabric layer. In this way the final product will have improved lightproof properties as the heating and optional addition of adhesive will ensure dimensional stability of the final screen product after assembly.

In a second aspect of the present invention, there is provided a screening arrangement for an aperture of a building structure, the screening arrangement comprising:
a top element arranged to be mountable to a top member of a window frame,
two side rails, and
a screening body according to the first aspect of the invention.

In a third aspect of the present invention, there is provided a method of manufacturing a screening body according to the first aspect of the present invention, the method comprising the steps of:
i. feeding a fabric layer to a guiding roll said fabric comprising an upper surface and a lower surface;
ii. contacting the fabric layer with an adhesive composition layer comprising thermoplastic polyurethane or polyethylene terephthalate to provide a combined fabric adhesive layer,
iii. heating the fabric adhesive layer to a temperature at which the adhesive softens, such as a temperature in the range of 120 ° to 180°C, preferably 130°C to 160°C, most preferred 145°C;
v. in successive steps optionally pre-heating an at least first coated metal strip comprising aluminium, the coating comprising epoxy;
vi. providing the, optionally heated, at least first metal strip to the upper surface of the fabric adhesive layer in successive steps extending in a longitudinal direction of the fabric adhesive layer;
vii. heating the fabric adhesive layer and the metal strip(s) to obtain the screening body.

Optionally, step vi. may comprise providing heated metal strips to each sides of the fabric adhesive layer. The adhesive may be applied to the bottom surface of the fabric layer.

In a preferred embodiment the adhesive is provided as a lined adhesive layer, whereby the liner is removed concurrently with laminating the adhesive layer to the fabric. It is also contemplated that the adhesive is provided as a liner less sheet or as a liquid. In further embodiments the adhesive is provided by extrusion, of e.g. a granulate, and said extruded adhesive is brought into contact with the fabric layer in step ii. The extrusion is preferably an integrated part of the method.

In yet a preferred embodiment the heating of step iii. and vii. takes place at the same temperature, preferably in the same heating unit.

In still an embodiment a cooling step is provided after step vii. the cooling is preferably to ambient temperature.

In a further embodiment the at least one metal strip is applied to the surface of the fabric at a distance of 1 to 8 mm, more preferred 2 to 5 mm, most preferred 3 mm.

In yet an embodiment the fabric layer is heated prior to being provided in step i. or an adhesive layer is provided to one or both sides of the fabric layer during heating and is preferably allowed to cool down prior to being provided in step i. The application of heat and/or a first adhesive to the fabric layer prior to assembly of the screen ensures dimensional stability of the fabric layer in the final product whereby the screen becomes more lightproof.

In embodiments where the adhesive layer applied in step ii. is applied on both sides of the fabric layer,the pressure applied in the lamination process is below 2 to 8 MPa, preferably 3-5 MPa, such as 4 MPa. By operating the lamination at reduced pressure the equipment will suffer less wear and hence last longer.

The method of manufacturing the screening body may in preferred embodiments vary in accordance with the variations of materials as detailed in the first aspect of the invention.

### Figures

Further details will be described and further advantages stated in the description of particular embodiments of the invention by reference to the accompanying drawings in which:
Fig.1 is an isometric view of a screening arrangement according to the present invention (part of the screening body has been removed for clarity);
Fig. 2 is an isometric view of a window comprising a screening arrangement with the window in a closed position and the screening body in a screening position (part of the screening body has been removed for clarity);
Figs. 3a - c is a cross sectional view of a screening body of the present invention;
Fig. 4 is a schematic representation of a manufacturing process according to the present invention; and
Fig. 5 is a schematic representation of an alternative manufacturing process according to the present invention;
Fig. 6 is a schematic representation of another alternative manufacturing process according to the present invention;
Fig. 7 is a graph showing results of a peel adhesion test comparing various embodiments of the invention with a conventional system.

### Detailed Description of the Invention

In the embodiment shown in Fig. 1, the screening arrangement in the form of a roller shutter 1 has a top element 2 and two side rails 3 and 4 extending at right angles to the top element 2. A shutter body 5 includes a plurality of slats 51, of which some have been omitted for clarity reasons only.

As shown in Fig. 2, the roller shutter 1 can be mounted on a window, for instance a roof window adapted for installation in an inclined roof. The window comprises in a manner known per se a window frame 6 and a window sash 7 encasing a pane 8. The window sash 7 will most often be openable relative to the window frame 6, viz. hinge connected to the window frame 6, for instance by means of a set of pivot hinges positioned close to a central axis of the window to allow the window sash 7 to pivot relative to the window frame 6, or by a more traditional hinge positioned at the top of the window. The aperture to be screened is defined by the area limited by the top element 2, the side rails 3, 4, and the bottom of the window. This aperture thus corresponds in substance to the pane 8.

In order to attain the desired screening, the shutter body 5 is adapted to be moved from a non-screening position to a screening position. In the screening position the shutter body 5 covers the pane 8 and other parts of the window to a larger or lesser degree. In the screening position shown in Fig. 2, the shutter body 5 has been rolled out to cover the entire aperture and defines a general screening plane.

The top element 2 is positioned at the top of the window and comprises in the embodiment shown a top cover 21 and two outer end covers, of which the right-hand end cover 22 is visible in Fig. 2. As will be described in further detail below, the top cover 21 and outer end 20 covers 22 serve to hide and protect the inner parts of the roller shutter 1, such as for instance the drive mechanisms for the rolling up and unrolling of the shutter body 5. Terms such as "left-hand" and "right-hand" refer to the orientation shown in for instance Fig. 2 and are utilized for reasons of convenience only.

The side rail 4 has a structure comprising parts that are movable relative to each other. In Fig. 2, only an outer side rail part 41 is visible. The side rail 4 has a bottom cover 40 at the bottom of the window. The side rails 3, 4 are connected to each other at the bottom part of the roller shutter 1, namely by a cross bar 35 connected to the 30 bottom cover 40 of side rail 4 and its counterpart bottom cover 30 of side rail 3. The cross bar 35 may for instance be riveted to each bottom cover 30, 40. The cross bar 35 (not shown in the detailed figures) contributes to the strength and resistance as well. However, the cross bar 35 is not strictly necessary, as sufficient strength may be provided by the side rails 3,4 themselves.

As can be seen from Fig. 2, each slat 51 extends in a longitudinal direction between two end edges and has first and second side edges parallel to the longitudinal direction, i.e. in parallel with the top element 2. The shutter body 5 is adapted to be wound up in and rolled out from the top element 2 by means of a driving device (not shown) in a direction perpendicular to said longitudinal direction to a first screening position.

A cross section of an exemplary embodiment of the screening body of the present invention is shown in Fig. 3a. The screening body 5 has an acrylic fabric layer 301 having a top surface 302 and a bottom surface 303. There is a thermoplastic polyurethane adhesive composition 304 on the bottom surface 303. Aluminium slats 305, 306 having an epoxy primer coating 307 on the surfaces facing the fabric are positioned adjacent the top and bottom surfaces 302, 303 of the fabric layer 301.

Figure 3b shows the adhesive 304 on the top surface 302 and Figure 3c shows the adhesive 304 on both the top and bottom surfaces 302, 303.

Acrylic fabric is well known to the skilled person. Acrylic fibers are synthetic fibers made from a polymer (polyacrylonitrile) with an average molecular weight of -100,000, about 1900 monomer units. For a fiber to be called "acrylic", the polymer generally must contain at least 85% acrylonitrile monomer. Typical comonomers are vinyl acetate or methyl acrylate. Acryl fabrics are generally available for example from Dickson under the tradename sunacryl.

The acrylic may be solution dyed and coated with an anti-smudge coating which results in very good weather resistance. It will be understood that any suitable fabric may be used in place of the acrylic fabric. For example, a polyester fabric may be used in place of the acrylic in the embodiment described above. Fabrics usable according the invention are obtainable from JM textiles under the name RO Allegro transparent or from Hunter Douglas under the name Baseline Dust Blocks and Green Screen Balance. Alternatively, a polyamide such as Kevlar ^{®} of DuPont may be used. The fabric layer may also be glass fiber or a glass fiber reinforced fabric. The fabric layer may be woven. In further embodiments where the fabric layer comprises glass fiber it may be non-coated or coated. In embodiments where the glass fiber is coated, the coating may be selected from but not limited to PVC or PU. Coated glas fiber reinforced fabric layers suitable according to the invention are available from i.a. Copaco or Phifer.

The fabric layer is preferably a square construction with the same mechanical performances in warp and weft directions.

In another embodiment or additionally the warp and weft densities are in the range of 30 and 6 ends respectively per cm, preferably 16-8 ends per cm.

The yarn used can have a linear mass density in the range of 76 - 540 dtex (i.e. mass in grams per 10,000 meters), preferable 167-420 dtex.

Such preferred yarns provide a more uniform surface which contibutes to better fixation and an improved lightproof screen.

It is preferred that the fabric surface is lean, meaning less hairy or complete free of loose single or bundles of loose filaments. The yarn in the fabric may be made of a staplefiber, preferably a combed version or multifilament or monofilament. In a particular embodiment the fabric weight is in the range of 80-300 g/m2, such as 100 to 200 g/m2.

The thermoplastic polyurethane is preferably aliphatic, such as Elastollan ^{®} of BASF Polyurethanes GmbH.

Even if the adhesive is applied to only one side of the acrylic (or other) fabric it can percolate through the material and can therefore adhere the metal slat on the top surface. It will be appreciated that any suitable adhesive may be used including the thermoplastic copolyester hotmelt film of Gerlinger Industries.

The coating is epoxy primer. Epoxy primers are known to the skilled person, suitable epoxy primers according to the present invention include DPLF Epoxy Primer available from Deltron, or similar and usable primers are available from Beckers. Preferred are aromatically based epoxy primers, such as high molecular weight epoxy resins based on Bisphenol A, more specifically 2,2-bis(p-glycidyloxyphenyl) propane condensation product with 2,2-bis(p-hydroxyphenyl) propane and similar isomers and/or phenol, 4,4'-(1-methylethylidene)bis-, polymer with 2,2'-[(1-methylethylidene)bis(4,1- phenyleneoxymethylene)] bis(oxirane) illustrated below by formula (I)

In the embodiment shown, the metal slats are made from EN AW-5754, which is an aluminium alloy having an aluminium content of greater than 90 wt%. In particular, it has the following composition: aluminium: 94.2 to 97.4%, chromium: 0.3% max, copper: 0.1% max, iron: 0.4% max, magnesium: 2.6 to 3.6%, manganese: 0.5% max, silicon: 0.4% max, titanium: 0.15% max, zinc: 0.2% max and 0.15% max of residuals. Suitable alternatives include EN AW-5006 and EN AW-3005, although any suitable metal known to the skilled person may be used. Particularly preferred are EN AW-5754 or EN AW-3005 having a good stability towards corrosion. Metal strips usable according to the present invention may be obtained from Elval or Novelis.

In an exemplary method of manufacturing the screening body 5 depicted in figure 4, a fabric layer 401 and an adhesive layer 402 are simultaneously fed to a guide roll 403 to produce a combined fabric adhesive layer 404. The adhesive layer 402 has a removable liner 405 which prevents the adhesive becoming stuck to the guide roll 403. Once the fabric layer 401 and adhesive layer 402 have passed through the guide roll 403 the liner 405 can be removed.

The combined fabric adhesive layer 404 can then be passed to a hot air oven 406. Here the adhesive softens and is thus primed for adhesion with further layers. It will be understood that the temperature to which the hot air oven should be heated will depend on the adhesive. Typically, a temperature in the range of around 120 ° to 180°C, preferably 130°C to 160°C, most preferred 145°C is appropriate. Rollers 407 can be used in the hot air oven 406. Alternatively and preferably, the heat is provided from the rollers 407 comprising a heating element.

Next, one or two preheated aluminium strips are brought into contact with the combined fabric adhesive layer. If one aluminium strip is used, it may be provided on the top or bottom surface of the combined fabric adhesive layer. If two aluminium strips are used, one will be provided on the top surface of the combined fabric adhesive layer and the other will be provided on the bottom surface said strips being provided to completely cover each other.

The aluminium strips are coated before the optional heating, preferably well before the manufacturing method to allow the coating to dry and cure.

The combined fabric adhesive layer 404 and aluminium layers 408, 409 are then passed through further rollers 410 and into a further hot air oven 411 where the combination is heated. Again, a temperature of around 145°C is typically suitable. Non-stick rollers 412 in the hot air oven 411 encourage the layers to adhere to one another and allow the screening body 5 formed to move through the hot air oven 411. A cooling section 414 can then be used to allow the adhesive to set. If necessary, the screening body can then be cut to shape.

In the alternative embodiment shown in Fig. 5, a fabric layer 501, an adhesive layer 502 and aluminium layers 508, 509 are simultaneously fed to a guide roll 510. The aluminium layers 508, 509 are coated before being introduced, preferably well before the manufacturing method to allow the coating to dry and cure.

The combination is then passed to a temperature controlled section 511 in which there is a heating section 520 and a cooling section 522. Whilst any suitable temperatures may be used, a temperature of around 120 ° to 180°C, preferably 130°C to 160°C, most preferred 145°C is typically appropriate for the heating section 520.

Guide rolls 512 allow the screening body formed to move through the temperature controlled section 511. In addition to guide rolls 512, there may be further rollers in the heating section 520 and/or the cooling section 522. Belts 525 and 526 may be used in the heating section 520 and/or the cooling section 522 to apply a constant pressure to the screening body 5, the pressure applied is typically around 18 MPa.

In the alternative embodiment shown in Fig. 6, a fabric layer 601 and adhesive layer 602 are simultaneously fed to first rolling section 603a. The first rolling section 603a comprises a first guide roll 603b and a second guide roll 603c separated by a heating portion 603d. The fabric layer 601 and adhesive layer 602 pass through the first guide roll 603b and are heated to soften the adhesive in heating portion 603d. One or more belts 603e may be used in the heating portion 603d to maintain the desired pressure. The fabric and adhesive then pass through second guide roll 603c and removable liner 605 is removed from the adhesive.

After the liner has been removed, an intermediate heater 630 is used to keep the adhesive at a temperature at which it is sticky but not molten. It will be understood that the specific temperature required to achieve this will depend on factors such as the type of adhesive used, although typically a temperature of around 70°C to 90°C is appropriate.

Aluminium layers 608 and 609 are fed with the fabric-adhesive combination to further rollers 610. Preheaters 632, 634 may be used to warm the aluminium sheets before they come into contact with the fabric. The combination is then passed to a temperature controlled section 611 in which there is a heating section 620 and a cooling section 622. Whilst any suitable temperatures may be used, a temperature of around 120 ° to 180°C, preferably 130°C to 160°C, most preferred 145°C is typically appropriate for the heating section 620.

Guide rolls 612 allow the screening body formed to move through the temperature controlled section 611. In addition to guide rolls 612, there may be further rollers in the heating section 620 and/or the cooling section 622. Belts may be used in the heating section 620 and/or the cooling section 622 to apply a constant pressure and/or heat to the screening body 5.

It will be understood that the aluminium strips are coated before heating, preferably well before the manufacturing method to allow the coating to dry and cure.

Different stages of the process may require different pressures. For example, the pressure applied by guide rolls 603b, 603c, 610 and 612 and any corresponding belts can be tailored according to the requirements of the process. In some embodiments, the pressure applied to the sample in the first rolling section 603a will be different from the pressure applied by the rollers 610 and/or the rollers 612.

The heat applied in heating portion 603d may be different from the heat applied by heating section 620. The temperature in these sections may be independently adjustable.

### Example 1

In order to test various embodiments of the screening body of the present invention and compare their characteristics with a conventional screening body, a peel test was conducted.

The peel test was carried out in accordance with the following industry standards: BS 5350-C12, ASTM D5170, ASTM F88 and ISO 11339.
Four embodiments were tested. Each had the structure outlined in Fig. 3, but with the materials selected as follows:

| | **Embodiment 1** | **Embodiment 2** | **Embodiment 3** | **Embodiment 4** |
|---|---|---|---|---|
| **Coating** | Epoxy | Polyethylene Terephthalate | Epoxy | Polyethylene Tere phthalate |
| **Fabric** | Acrylic | Acrylic | Acrylic | Acrylic |
| **Adhesive** | Thermoplastic Polyurethane | Thermoplastic Polyurethane | Polyethylene Terephthalate | Polyethylene Terephthalate |
| **Metal** | Aluminium | Aluminium | Aluminium | Aluminium |

The performance of the embodiments were compared with that of a commercially available product in which the fabric was poly ethylenetere phthalate (PET), the fabric layer polyethylene and an adhesive (not known).

A number of tests were conducted under a variety of conditions intended to replicate the conditions that a screening body may encounter during use

| **Stress factors** | **Degradation mechanisms** | **Accelerated tests** |
|---|---|---|
| Elevated temperature. Screening body can reach 80-85°C | Speed up degradation process of hydrolysis, oxidation etc. | Climate test @ 85°C, 80% RH Florida test* (peel test) |
| Moisture/water The fabric and adhesive absorb water | Hydrolysis of adhesive, fabric and primer. Water react with polymer and break down the polymer chain | Climate test @85°C, 80 % RH |
| | | Xenon test |
| | | Florida test |
| | | Water emission test |
| Low temperature. Water freezes to ice | Water expansion. Stress the construction and the adhesive interface | Cataplasmatest 70°C, 100 %RH to -20°C |
| UV radiation | Polymer degradation. Stimulate the oxidation process, creates free radicals and can lead to polymer chain breaks | Xenon test |
| | | QUV B |
| | | Florida test |

Tests indicated with "*" are future suitable tests to be performed

To provide a comparison, the peel test was also conducted when no ageing process was applied to the samples.

The results of the peel test can be found in Fig. 7.

As can be seen, the samples were able to withstand a greater load under at least some of the test conditions compared with the commercially available sample. Some of the samples, namely those of embodiments 1 and 3, were able to withstand a greater average load than the commercially available system in all of the tests. Thus, it is apparent that these samples have stronger adhesion characteristics and are more resistant to delamination. They would therefore exhibit a longer useable lifetime than the conventional system tested.

### Example 2

Following the initial peel test, further tests were conducted. Additional embodiments were tested which were analogous to those of embodiments 1 and 3, but with a polyester rather than an acrylic fabric. The tested embodiments were as follows:

| | **Embodiment 1** | **Embodiment 3** | **Embodiment 5** | **Embodiment 6** |
|---|---|---|---|---|
| **Coating** | Epoxy | Epoxy | Epoxy | Epoxy |
| **Fabric** | Acrylic | Acrylic | Polyester | Polyester |
| **Adhesive** | Thermoplastic Polyurethane | Polyethylene Terephthalate | Thermoplastic Polyurethane | Polyethylene Terephthalate |
| **Metal** | Aluminium | Aluminium | Aluminium | Aluminium |

A general summary of the results can be found in the table below. The number 1 represents a positive result, 2 represents a need for further investigation and 3 represents a result under average. The score was based on an overall evaluation of the sum of parameters and properties tested.

| | **Embodiment 1** | **Embodiment 3** | **Embodiment 5** | **Embodiment 6** | **Commerically available product** |
|---|---|---|---|---|---|
| **Adhesion and Delamination** | *1* | *2* | *2* | *3* | *3* |
| **UV Stability** | *1* | *2* | *2* | *2* | *2* |
| **Black-out** | *1* | *1* | *1* | *1* | *1* |
| **Resist surface temperatures of -25°C to 80°C** | *1* | *1* | *1* | *1* | *1* |
| **Resist humidity** | *1* | *3* | *3* | *3* | *3* |
| **Process (producible)** | *1* | *1* | *1* | *1* | *-* |

Particularly favorable characteristics were observed for embodiment 1. This embodiment has the structure shown in Fig. 3 with aluminium metal layers, an epoxy coating on the aluminium, acrylic fabric and an aliphatic thermoplastic polyurethane adhesive. Embodiment 5, in which the structure is identical to embodiment 3 except that the fabric is polyester rather than acrylic, also showed surprisingly positive results.

## Claims

1. A screening body (5) for a screening arrangement (1) including a top element (2) defining a longitudinal direction, said screening body (5) comprising a plurality of slats (51) and a fabric layer (301) having a top surface (302) and a bottom surface (303), each slat (51) extending in a longitudinal direction between two end edges and having first and second side edges parallel to the longitudinal direction, the screening body (5) being adapted to be wound up in and rolled out from said top element (2) in a direction perpendicular to said longitudinal direction to a screening position in which the screening body defines a general screening plane; in which each of the slats (51) is composed of at least one metal strip (305) connected to the fabric layer (301), wherein the at least one first metal strip (305) comprises aluminium, wherein
the at least one metal strip is coated with a coating (307) on at least the side facing the fabric layer (301) and an adhesive layer (304) binds the metal strip (305) to the fabric layer (301);
the screening body (5) being **characterised in that**
the coating (307) comprises epoxy,
wherein the adhesive composition of the adhesive layer (304) comprises thermoplastic polyurethane or polyethylene terephthalate.

2. A screening body (5) according to claim 1, wherein the at least first metal strip is arranged to contact the top surface (302) of the fabric layer (301) and a second metal strip is arranged to contact the bottom surface (303) of the fabric layer (301).

3. A screening body (5) according to claim 1, wherein the at least one metal strip comprises an alloy having an Al content in an amount of at least 90 wt% or more preferably at least 93 wt%, most preferred at least 95%.

4. A screening body (5) according to any one of the preceding claims, wherein the coating (307) is an aromatically based epoxy.

5. A screening body (5) according to any one of the preceding claim, wherein the adhesive composition comprises an aliphatic thermoplastic polyurethane, more preferred an aliphatic polyether polyurethane

6. A screening body (5) according to anyone of the preceding claims, wherein the adhesive layer (304) has been applied to the bottom surface of the fabric layer.

7. A screening body (5) according to any one of the preceding claims, wherein the adhesive composition additionally comprises and/or is a UV stabiliser.

8. A screening body (5) according to any one of the preceding claims, wherein the fabric layer (301) comprises acrylic, polyester, glass fiber, a glass fiber reinforced layer or a polyamide.

9. A screening body (5) according to any of the preceding claims, wherein the fabric layer (301) comprises acrylic or polyester, the at least one first metal strips comprises an alloy having an aluminium content in an amount of at least 90 wt%, the adhesive composition comprises a thermoplastic polyurethane and the coating comprises epoxy.

10. A screening arrangement (1) for an aperture of a building structure, the screening arrangement comprising:
a top element (2) arranged to be mountable to a top member of a window frame (6),
two side rails (3,4), and
a screening body (5) according to any one of the preceding claims.

11. A method of manufacturing a screening body (5) according to any of the claims 1 to 9, the method comprising the steps of:
i. feeding a fabric layer (301) to a guiding roll (403) said fabric comprising a top surface and a bottom surface;
ii. contacting the fabric layer (301) with an adhesive composition layer (304) comprising thermoplastic polyurethane or polyethylene terephthalate to provide a combined fabric adhesive layer
iii. heating the fabric adhesive layer to a temperature at which the adhesive softens, such as a temperature in the range of 120 ° to 180°C, preferably 130°C to 160°C, most preferred 145°C;
v. in successive steps optionally pre-heating an at least first coated metal strip comprising aluminium, the coating comprising epoxy;
vi. providing the, optionally heated, at least first metal strip to the upper surface of the fabric adhesive layer in successive steps extending in a longitudinal direction of the fabric adhesive layer;
vii. heating the fabric adhesive layer and the metal strip(s) to obtain the screening body.

12. Method according to claim 11, wherein step vi. comprises providing heated metal strips to each sides of the fabric adhesive layer.

13. Method according to claim 11 or 12, wherein the adhesive layer is applied to the bottom surface of the fabric layer.

14. Method according to any one of claims 11 to 13, wherein the adhesive layer (304) is provided as a lined adhesive layer or wherein the adhesive layer (304) is provided by extrusion immediately prior to being contacted with the fabric layer in step ii.

15. Method according to any one of claims 11 to 14, wherein the heating of step iii. and vii. takes place at the same temperature, preferably in the same heating unit.

16. Method according to any one of claims 11 to 15, wherein the method further comprises the step of cooling the fabric adhesive layer and the metal strip(s) after they have been heated in step vii.

17. Method according to any one of claims 11 to 16, wherein the method is flatbed lamination.

18. Method according to any one of claims 11 to 17, wherein the fabric layer is heated prior to being provided in step i. or wherein an adhesive is applied to the fabric under heating prior to being provided in step i.

19. Method according to any one of claims 11 to 18, wherein the adhesion layer is applied to both the bottom and top surfaces of the fabric layer (301) and wherein the pressure applied in the lamination process is below 100 bar, such as below 50 bar.

## Patentansprüche

1. Abschirmkörper (5) für eine Abschirmanordnung (1), die ein oberes Element (2) einschließt, das eine Längsrichtung definiert, wobei der Abschirmkörper (5) eine Vielzahl von Lamellen (51) und eine Stoffschicht (301) mit einer oberen Oberfläche (302) und einer unteren Oberfläche (303) umfasst, wobei jede Lamelle (51) sich zwischen zwei Endkanten in einer Längsrichtung erstreckt und erste und zweite Seitenkanten parallel zu der Längsrichtung aufweist, wobei der Abschirmkörper (5) eingerichtet ist, um von dem oberen Element (2) aus in einer Richtung rechtwinklig zu der Längsrichtung aufgewickelt und auf eine Abschirmposition abgerollt zu werden, in der der Abschirmkörper eine allgemeine Abschirmebene definiert; wobei jede der Lamellen (51) aus mindestens einem Metallstreifen (305) zusammengesetzt ist, der mit der Stoffschicht (301) verbunden ist, wobei der mindestens eine erste Metallstreifen (305) Aluminium umfasst,
wobei der mindestens eine Metallstreifen mit einer Beschichtung (307) auf mindestens der Seite, die zu der Stoffschicht (301) weist, beschichtet ist, und eine Klebeschicht (304) den Metallstreifen (305) an die Stoffschicht (301) bindet;
wobei der Abschirmkörper (5) **dadurch gekennzeichnet ist, dass**
die Beschichtung (307) Epoxy umfasst,
wobei die Klebezusammensetzung der Klebeschicht (304) thermoplastisches Polyurethan oder Polyethylenterephthalat umfasst.

2. Abschirmkörper (5) nach Anspruch 1, wobei der mindestens erste Metallstreifen vorgesehen ist, um die obere Oberfläche (302) der Stoffschicht (301) zu kontaktieren, und ein zweiter Metallstreifen vorgesehen ist, um die untere Oberfläche (303) der Stoffschicht (301) zu kontaktieren.

3. Abschirmkörper (5) nach Anspruch 1, wobei der mindestens eine Metallstreifen eine Legierung mit einem Al-Gehalt in einer Menge von mindestens 90 Gew.% oder mehr, vorzugsweise mindestens 93 Gew.%, am meisten bevorzugt mindestens 95 % umfasst.

4. Abschirmkörper (5) nach einem der vorhergehenden Ansprüche, wobei die Beschichtung (307) ein Epoxy auf aromatischer Basis ist.

5. Abschirmkörper (5) nach einem der vorhergehenden Ansprüche, wobei die Klebezusammensetzung ein aliphatisches thermoplastisches Polyurethan, bevorzugter ein aliphatisches Polyetherpolyurethan umfasst.

6. Abschirmkörper (5) nach einem der vorhergehenden Ansprüche, wobei die Klebeschicht (304) auf die untere Oberfläche der Stoffschicht aufgebracht worden ist.

7. Abschirmkörper (5) nach einem der vorhergehenden Ansprüche, wobei die Klebezusammensetzung zusätzlich einen UV-Stabilisator umfasst und/oder ein solcher ist.

8. Abschirmkörper (5) nach einem der vorhergehenden Ansprüche, wobei die Stoffschicht (301) Acryl, Polyester, Glasfaser, eine glasfaserverstärkte Schicht oder ein Polyamid umfasst.

9. Abschirmkörper (5) nach einem der vorhergehenden Ansprüche, wobei die Stoffschicht (301) Acryl oder Polyester umfasst, der mindestens eine erste Metallstreifen eine Legierung mit einem Aluminiumgehalt in einer Menge von mindestens 90 Gew.% umfasst, die Klebezusammensetzung ein thermoplastisches Polyurethan umfasst und die Beschichtung Epoxy umfasst.

10. Abschirmanordnung (1) für einen Durchbruch einer Gebäudestruktur, wobei die Abschirmanordnung umfasst:
ein oberes Element (2), das vorgesehen ist, um an einem Oberteil eines Fensterrahmens (6) montierbar zu sein,
zwei Seitenschienen (3, 4), und
einen Abschirmkörper (5) nach einem der vorhergehenden Ansprüche.

11. Verfahren zum Fertigen eines Abschirmkörpers (5) nach einem der Ansprüche 1 bis 9, wobei das Verfahren die Schritte umfasst:
i. Zuführen einer Stoffschicht (301) zu einer Führungsrolle (403), wobei der Stoff eine obere Oberfläche und eine untere Oberfläche umfasst;
ii. Kontaktieren der Stoffschicht (301) mit einer Klebezusammensetzungsschicht (304), die thermoplastisches Polyurethan oder Polyethylenterephthalat umfasst, um eine kombinierte Stoff-Klebeschicht bereitzustellen,
iii. Erwärmen der Stoff-Klebeschicht auf eine Temperatur, bei der der Klebstoff weich wird, wie eine Temperatur im Bereich von 120 ° bis 180 °C, vorzugsweise 130 °C bis 160 °C, am meisten bevorzugt 145 °C;
v. in aufeinander folgenden Schritten gegebenenfalls Vorheizen von mindestens einem ersten beschichteten Metallstreifen, der Aluminium umfasst, wobei die Beschichtung Epoxy umfasst;
vi. Bereitstellen des gegebenenfalls erwärmten mindestens ersten Metallstreifens, der sich in einer Längsrichtung der Stoff-Klebeschicht erstreckt, an die obere Oberfläche der Stoff-Klebeschicht in aufeinander folgenden Schritten;
vii. Erwärmen der Stoff-Klebeschicht und des Metallstreifens/der Metallstreifen, um den Abschirmkörper zu erhalten.

12. Verfahren nach Anspruch 11, wobei Schritt vi. Bereitstellen von erwärmten Metallstreifen an jede Seite der Stoff-Klebeschicht umfasst.

13. Verfahren nach Anspruch 11 oder 12, wobei die Klebeschicht auf die untere Oberfläche der Stoffschicht aufgebracht wird.

14. Verfahren nach einem der Ansprüche 11 bis 13, wobei die Klebeschicht (304) als Klebeschichtauskleidung bereitgestellt wird, oder wobei die Klebeschicht (304) durch Extrusion bereitgestellt wird, unmittelbar bevor sie mit der Stoffschicht in Schritt ii. kontaktiert wird.

15. Verfahren nach einem der Ansprüche 11 bis 14, wobei das Erwärmen von Schritt iii. und vii. auf die gleiche Temperatur, vorzugsweise in der gleichen Heizeinheit stattfindet.

16. Verfahren nach einem der Ansprüche 11 bis 15, wobei das Verfahren des Weiteren den Schritt des Kühlens der Stoff-Klebeschicht und des Metallstreifens/der Metallstreifens umfasst, nachdem sie in Schritt vii. erwärmt worden sind.

17. Verfahren nach einem der Ansprüche 11 bis 16, wobei das Verfahren Flachbettlaminierung ist.

18. Verfahren nach einem der Ansprüche 11 bis 17, wobei die Stoffschicht erwärmt wird, bevor sie in Schritt i. bereitgestellt wird, oder wobei ein Klebstoff auf den Stoff unter Erwärmen aufgebracht wird, bevor die Bereitstellung in Schritt i. erfolgt.

19. Verfahren nach einem der Ansprüche 11 bis 18, wobei die Klebeschicht auf sowohl die untere als auch auf die obere Oberfläche der Stoffschicht (301) aufgebracht wird, und wobei der in dem Laminierungsprozess angewendete Druck unter 100 bar, wie unter 50 bar, liegt.

## Revendications

1. Corps de protection (5) pour un agencement de protection (1) comportant un élément supérieur (2) définissant une direction longitudinale, ledit corps de protection (5) comprenant une pluralité de lames (51) et une couche de tissu (301) ayant une surface supérieure (302) et une surface inférieure (303), chaque lame (51) s'étendant dans une direction longitudinale entre deux bords d'extrémité et ayant des premier et deuxième bords latéraux parallèles à la direction longitudinale, le corps de protection (5) étant adapté pour être enroulé dans ledit et déroulé dudit élément supérieur (2) dans une direction perpendiculaire à ladite direction longitudinale jusqu'à une position de protection dans laquelle le corps de protection définit un plan de protection générale, dans lequel chacune des lames (51) est composée d'au moins une bande métallique (305) reliée à la couche de tissu (301), dans lequel l'au moins une bande métallique (305) comprend de l'aluminium,
dans lequel l'au moins une bande métallique est recouverte d'un revêtement (307) au moins sur le côté faisant face à la couche de tissu (301) et une couche d'adhésif (304) lie la bande métallique (305) à la couche de tissu (301) ;
le corps de protection (5) étant **caractérisé en ce que**
le revêtement (307) comprend de la résine époxy,
dans lequel la composition d'adhésif de la couche d'adhésif (304) comprend du polyuréthane thermoplastique ou du téréphtalate de polyéthylène.

2. Corps de protection (5) selon la revendication 1, dans lequel l'au moins une première bande métallique est disposée pour être en contact avec la surface supérieure (302) de la couche de tissu (301) et une deuxième bande métallique est disposée pour être en contact avec la surface inférieure (303) de la couche de tissu (301).

3. Corps de protection (5) selon la revendication 1, dans lequel l'au moins une bande métallique comprend un alliage ayant une teneur en Al dans une quantité d'au moins 90 % en poids ou mieux au moins 93 % en poids, idéalement au moins 95 %.

4. Corps de protection (5) selon l'une quelconque des revendications précédentes, dans lequel le revêtement (307) est une résine époxy à base aromatique.

5. Corps de protection (5) selon l'une quelconque des revendications précédentes, dans lequel la composition d'adhésif comprend un polyuréthane thermoplastique aliphatique, mieux un polyuréthane de polyéther aliphatique.

6. Corps de protection (5) selon l'une quelconque des revendications précédentes, dans lequel la couche d'adhésif (304) a été appliquée à la surface inférieure de la couche de tissu.

7. Corps de protection (5) selon l'une quelconque des revendications précédentes, dans lequel la composition d'adhésif comprend également et/ou est un stabilisant UV.

8. Corps de protection (5) selon l'une quelconque des revendications précédentes, dans lequel la couche de tissu (301) comprend de la résine acrylique, du polyester, de la fibre de verre, une couche renforcée de fibres de verre ou un polyamide.

9. Corps de protection (5) selon l'une quelconque des revendications précédentes, dans lequel la couche de tissu (301) comprend de la résine acrylique ou du polyester, l'au moins une première bande métallique comprend un alliage ayant une teneur en aluminium dans une quantité d'au moins 90 % en poids, la composition d'adhésif comprend un polyuréthane thermoplastique et le revêtement comprend de la résine époxy.

10. Agencement de protection (1) pour une ouverture d'une structure de bâtiment, l'agencement de protection comprenant :
un élément supérieur (200) agencé pour pouvoir être monté sur un élément supérieur d'un châssis de fenêtre (6),
deux rails latéraux (3, 4), et
un corps de protection (5) selon l'une quelconque des revendications précédentes.

11. Procédé de fabrication d'un corps de protection (5) selon l'une quelconque des revendications 1 à 9, le procédé comprenant les étapes suivantes :
i. avance d'une couche de tissu (301) jusqu'à un rouleau de guidage (403), ledit tissu comprenant une surface supérieure et une surface inférieure ;
ii. mise en contact de la couche de tissu (301) avec une couche de composition d'adhésif (304) comprenant du polyuréthane thermoplastique ou du téréphtalate de polyéthylène pour fournir une couche combinée de tissu-adhésif ;
iii. chauffage de la couche de tissu-adhésif jusqu'à une température à laquelle l'adhésif se ramollit, telle qu'une température dans la plage de 120° à 180 °C, de préférence 130 °C à 160 °C, idéalement 145 °C ;
v. dans des étapes successives, éventuellement, préchauffage d'au moins une première bande métallique revêtue comprenant de l'aluminium, le revêtement comprenant de la résine époxy ;
vi. fourniture de l'au moins une première bande métallique, éventuellement chauffée, à la surface supérieure de la couche de tissu-adhésif dans des étapes successives s'étendant dans une direction longitudinale de la couche de tissu-adhésif ;
vii. chauffage de la couche de tissu-adhésif et de la/des bande(s) métallique(s) pour obtenir le corps de protection.

12. Procédé selon la revendication 11, dans lequel l'étape vi. comprend la fourniture de bandes métalliques chauffées à chaque côté de la couche de tissu-adhésif.

13. Procédé selon la revendication 11 ou 12, dans lequel la couche d'adhésif est appliquée à la surface inférieure de la couche de tissu.

14. Procédé selon l'une quelconque des revendications 11 à 13, dans lequel la couche d'adhésif (304) est fournie sous la forme d'une couche d'adhésif doublée ou dans lequel la couche d'adhésif (304) est fournie par extrusion juste avant d'être mise en contact avec la couche de tissu à l'étape ii.

15. Procédé selon l'une quelconque des revendications 11 à 14, dans lequel le chauffage des étapes iii. et vii. a lieu à la même température, de préférence dans la même unité de chauffage.

16. Procédé selon l'une quelconque des revendications 11 à 15, le procédé comprenant en outre l'étape de refroidissement de la couche de tissu-adhésif et de la/des bande(s) métallique(s) après qu'elles ont été chauffées à l'étape vii.

17. Procédé selon l'une quelconque des revendications 11 à 16, le procédé étant une stratification à plat.

18. Procédé selon l'une quelconque des revendications 11 à 17, dans lequel la couche de tissu est chauffée avant d'être fournie à l'étape i. ou dans lequel un adhésif est appliqué au tissu sous chauffage avant d'être fourni à l'étape i.

19. Procédé selon l'une quelconque des revendications 11 à 18, dans lequel la couche d'adhésif est appliquée à la fois aux surfaces inférieure et supérieure de la couche de tissu (301) et dans lequel la pression appliquée dans l'opération de stratification est inférieure à 100 bar, par exemple inférieure à 50 bar.
